

## UNITED STATES PATENT OFFICE

GEORGE A. RICHTER, OF BERLIN, NEW HAMPSHIRE, ASSIGNOR TO BROWN COMPANY, OF  
BERLIN, NEW HAMPSHIRE, A CORPORATION OF MAINE

## PROCESS OF LOWERING THE SOLUTION VISCOSITY OF CELLULOSE FIBER

No Drawing.

Application filed August 22, 1928. Serial No. 301,442.

In the manufacture of various cellulose products such as artificial silk, lacquers, and fibers, it is the practice to convert cellulose fiber into a derivative such as xanthate, nitrate, or acetate, and then to dissolve the derivative in a suitable solvent or mixture of solvents before forming into the ultimate product. In order to produce solutions of a viscosity sufficiently low to permit spinning into silk filaments, or use as lacquers, or forming into films, it is necessary either to depolymerize to lower the solution viscosity of the fiber used as a raw material, or to treat the derivative prepared therefrom in a manner to lower its solution viscosity. In the viscose-rayon industry, for example, depolymerization of the fiber is effected by soaking sheets of fiber with a caustic soda solution of mercerizing strength, pressing the sheets free of excess solution and disintegrating them into a fluffy mass, and finally ageing the mass for a considerable period of time. Not only is such a process time-consuming and expensive, but the ageing conditions must be carefully controlled to prevent degradation of the fiber into oxyzcelluloses and other undesirable reaction products. When the derivative is treated to lower its solution viscosity, as nitrocellulose sometimes is, under heat and pressure, not only must it be handled in comparatively small batches, but the treatment must also be carefully controlled to prevent decomposition from taking place.

One of the objects of the present invention is to provide a process for markedly and rapidly lowering the solution viscosity of cellulose fiber while it is in the form of an aqueous pulp of, say, about 2% to 10% fiber content, as this permits easy and continuous handling of large amounts of fiber by the use of comparatively inexpensive apparatus. Another object is to effect a lowering of the solution viscosity of cellulose fiber substantially without affecting its alpha cellulose content so that the product is unimpaired in value for use as a raw material for the preparation of high grade derivatives. Still another object is to effect such solution viscosity lowering of cellulose fiber without impairing the capacity of such fiber undergoing hydration or gelatinization when beaten (when such impairment is undesirable), so that the resulting fiber may be successfully sheeted on paper machines into tissues or waterleaf papers suitable for nitration, acetylation, or other chemical conversion.

The term "solution viscosity" as applied to cellulose fiber is an arbitrary one, being indicative of the viscosity of a cellulose derivative solution preparable therefrom. The solution employed as a standard is a cuprammonium cellulose solution of prescribed cellulose concentration, the viscosity being determined by measuring the viscosity of a definite volume of such solution under standard conditions, through an orifice of standard size. The solution viscosity of fiber is herein given in absolute C. G. S. units, and is determined by measuring the viscosity of a solution of 6 grams of fiber in a cuprammonium solution composed of 225 cc. of 28% ammonia water containing 9 grams of cuprous oxide. The C. G. S. unit is employed

because it is definite, denoting a viscosity 100 times that of water at 20° C., wherefore a cuprammonium cellulose solution of standard composition identifying a fiber as having a solution viscosity of 10 is 1000 times as 55 viscous as water at 20° C. Glycerine, which is often referred to when dealing with viscosity, for example, has a value of between 8 and 10 units.

One of the objects of the present invention is to provide a process for markedly and rapidly lowering the solution viscosity of cellulose fiber while it is in the form of an aqueous pulp of, say, about 2% to 10% fiber content, as this permits easy and continuous handling of large amounts of fiber by the use of comparatively inexpensive apparatus. Another object is to effect a lowering of the solution viscosity of cellulose fiber substantially without affecting its alpha cellulose content 60 so that the product is unimpaired in value for use as a raw material for the preparation of high grade derivatives. Still another object is to effect such solution viscosity lowering of cellulose fiber without impairing the capacity 65 of such fiber undergoing hydration or gelatinization when beaten (when such impairment is undesirable), so that the resulting fiber may be successfully sheeted on paper machines into tissues or waterleaf papers 70 suitable for nitration, acetylation, or other chemical conversion.

I have discovered that these objects may be attained by oxygenating cellulose fiber while suspended in an alkaline aqueous solution under a pressure of oxygenating gas materially greater than the vapor pressure of the solution. As a matter of practice, the alkaline aqueous suspension of fiber may be confined in a digester in contact with an atmosphere of oxygenating gas such as air or oxygen under the desired pressure. Preferably, the suspension is agitated during the treatment, as this exposes fresh surfaces of fiber to the action of the gas and tends to 80 produce a more rapid and uniform action. Apparently the comparatively high concentration of oxygen in the gas phase above the suspension brings about the desired results, 85 for in the course of experiments leading up 90 to

100

to the present discovery, it was found impossible to obtain a marked lowering of solution viscosity of the fiber by digesting the suspension at elevated temperatures in open tanks or by digesting in closed digesters under steam pressure. Even when air or oxygen is bubbled through the suspension in open tanks, reduction in the solution viscosity of the fiber takes place so slowly that one cannot obtain a product having a solution viscosity below 1, which is especially desired when the fiber is used as a raw material in the manufacture of cellulose products of the character described, in a reasonable and practical period of time.

In carrying out the process of the present invention, it is preferable to raise the temperature of the suspension, as this accelerates the reaction, but in so doing care must be exercised not to exceed the temperature at which the alpha cellulose content of the fiber is lowered and the yield of product seriously diminished. Metal compounds, such as those of iron, nickel, cobalt, manganese, and vanadium, when introduced into the alkaline solution, also tend to accelerate the reaction.

Cellulose fibers of various origins may be employed as a raw material. For example, one may start with white wood fiber refined to an alpha cellulose content of about 94% and having a solution viscosity of about 5 to 9, with cotton fiber as long staple, cotton linters, or rag pulp, and having a solution viscosity of 5 to 50, or with chemical wood pulp such as bleached sulphite pulp having an alpha cellulose content of about 86% and a solution viscosity of about 5 to 7. One may also employ incompletely refined wood pulps such as unbleached refined sulphite pulp or raw pulps such as unbleached unrefined sulphite or even kraft pulp.

A better appreciation of the process of the present invention may be gained from the following specific example. A refined wood pulp having an alpha cellulose content of 94.5% and a solution viscosity of 6 was employed as a raw material. The pulp was mixed with a 1% caustic soda solution to produce a 4% pulp suspension, which was confined in a digester under an air pressure of 100 pounds. While being maintained under this pressure, the suspension was subjected to agitation and its temperature raised to 130° F. At the end of a four-hour treatment under these conditions, it was noted that the solution viscosity of the fiber had been lowered to about 0.6, while its alpha cellulose content had remained substantially unchanged. The product may be washed free of alkaline solution, after which it may be dried in bulk form, or beaten and sheeted on a paper machine.

The foregoing example is illustrative of a rather wide range of conditions under which the treatment may be carried out, depending

upon the character of the raw material, the product which it is desired to produce, and the time in which it is desired to produce the product. For instance, the temperature of treatment may be lower, say 100° F., but with lower temperature a longer treatment is necessary in order to attain the desired solution viscosity of fiber. It is preferable to carry out the treatment below 150° F., in the case of a wood pulp of high alpha cellulose content such as herein before described, for should this temperature be exceeded, a drop in the yield and sometimes in the alpha cellulose content of the product is likely to result. Thus, when a treatment was carried out substantially according to the example hereinbefore described, but at a temperature of 200° F., it was found that a reduction of the solution viscosity of the fiber to about 0.6 resulted in a product of an alpha cellulose content of about 92%. The air pressure under which the suspension is confined may be as low as about 20 pounds, but a longer treatment is necessary in order to attain the desired viscosity. Oxygen gas, when economically available, may be advantageously used in place of air, as the desired solution viscosity of the fiber may be attained in a shorter period of time. The alkalinity of the solution and the density of the pulp suspension may be varied, but too high a pulp density should be avoided so as to permit adequate contact of oxygen and fiber during agitation. When mercerization of the fiber is not objectionable, as when the product is to be converted in bulk form into the xanthate, the fiber may be suspended in solutions of mercerizing alkalinity, in which case the treatment may be effected at comparatively low temperature, say, 40° to 70° F., to produce a product of a given low solution viscosity in a certain period of time. Caustic potash or other alkalies may be employed in place of caustic soda, but with weaker alkalies such as sodium carbonate, tri-sodium phosphate, and lime, a longer treatment is necessary in order to effect a given viscosity lowering.

The resulting product may have an alpha cellulose content higher than that of the original stock. Thus, if stocks, such as sulphite pulp are employed, it is likely that the fiber will undergo an increase in alpha cellulose content, owing to the solution of non-alpha cellulose components such as ligneous matter and beta and gamma celluloses from the pulp. The product may have a solution viscosity of from 0.3 to 1.0, depending upon the condition of treatment, and when mercerized is especially suitable for conversion into viscose, as no ageing is required to depolymerize a soda cellulose prepared therefrom. The product also has a lower copper number and a lower soda solubility (i. e., content of material dissolved by boiling in a 7% 125

caustic soda solution for one hour), showing that the fiber, rather than being degraded, is improved in its characteristics for conversion into cellulose derivatives. Thus, in 5 the specific example hereinbefore given, the refined wood pulp used as a raw material had a copper number of 1.5 and a soda solubility of 9, and resulted in a product having a copper number of 1.0 and a soda solubility of 5.

10 If the effect of the treatment is accelerated by introducing compounds of iron into the alkaline solution in which the fiber is suspended, or if the treatment is carried out in iron receptacles, the fiber will be stained by 70 iron compounds. If the fiber is but slightly stained, as when the treatment is carried out at comparatively low temperatures in iron receptacles, treatment of the fiber with a dilute solution of sulphurous acid will 75 restore the original color of the fiber, but if more markedly stained, the original color may be restored by digesting for a comparatively short time in a weak solution of oxalic acid.

25 When an unbleached wood fiber is employed as a raw material, the bleaching of such fiber may be advantageously combined with a treatment such as herein described. For instance, assuming unbleached, refined 30 wood fiber, which requires a comparatively small amount of bleach to be whitened, to be the raw material, such fiber may be treated as a 4% to 8% pulp suspension in, say, a 1% caustic soda solution containing, say, about 35 2% bleach based on dry weight of fiber, the treatment being carried out at, or slightly above, room temperature, for about six to ten hours. The bleach is substantially consumed in this treatment, but the whitened stock remains in a distinctly alkaline condition, and when raised to a temperature of about 130° F. and subjected to an air pressure of about 100 pounds for about four to six hours, resulted in a product having a low solution 40 viscosity, such as hereinbefore described. One of the advantages of a treatment thus carried out is that the caustic soda serves two purposes, namely, that of maintaining the stock in a distinctly alkaline condition during the bleaching operation, and so avoiding the formation of oxycelluloses and other degradation products, and also that of maintaining the stock in the desired alkaline condition during the subsequent treatment for 45 reducing its solution viscosity.

If a product of exceedingly low solution viscosity, say, 0.1, or lower, is desired, a treatment such as herein described may be advantageously combined with a process such 50 as described in patent application Serial No. 132,319, filed August 28, 1926. According to that process, cellulose fiber is first depolymerized by first treating such fiber as in the form of sheets with a caustic soda solution of 55 mercerizing strength, then pressing free of excess solution, and allowing the fiber (the so-called "soda cellulose") to age until the desired depolymerization and reduction in solution viscosity of fiber has taken place. The aged fiber is then washed to remove undesirable water-soluble constituents therefrom, and preferably then digested in an alkaline solution to remove undesirable water-insoluble constituents such as oxycelluloses. The process of that patent application 60 may, for instance, be applied to convert a refined wood fiber having an alpha cellulose content of, say, about 94% and a solution viscosity of about 6 into a final product having an alpha cellulose content of 65 about 95% to 96% and a solution viscosity of about 0.4 to 0.5, but should ageing be effected under conditions resulting in a product having a solution viscosity as low as .1, the alpha cellulose content and yield of the product 70 are likely to be seriously decreased. By further treating the fiber of low solution viscosity produced in accordance with the process therein described, in accordance with my present process these undesirable results may 75 be avoided. For instance, a fiber having an alpha cellulose content of about 95% to 96% and a solution viscosity of about 0.4 to 0.5, when treated with 1% NaOH solution at 30° F. and at 100 pounds air pressure, results in 80 a final product having an alpha cellulose content of about 95% to 97% and a solution viscosity of about 0.1 or lower. Such a product is of advantage, for instance, when it is desired to increase the cellulose concentration 85 in a viscose solution without increasing the caustic soda required to maintain the cellulose in solution, thereby lowering the caustic soda consumption and the acid consumption in the filament setting baths. For instance, 90 whereas it may be necessary to use a 6.5% caustic soda solution to maintain 7% cellulose in solution in usual practice, when a fiber having a solution viscosity of, say, .1 is employed as a raw material, it may not be necessary to use more caustic soda to keep in the 95 order of magnitude of 15% cellulose in solution.

There may be other changes or modifications in the process hereinbefore described, 100 which will suggest themselves to those skilled in the art, without departing from the spirit or scope of invention as defined in the appended claims.

What I claim is:

1. A process which comprises oxygenating a suspension of cellulose fiber in the physical condition of pre-liberated wood pulp in an alkaline aqueous solution under a pressure of oxygenating gas materially greater than 105 the vapor pressure of the solution.
2. A process which comprises oxygenating a suspension of cellulose fiber in the physical condition of pre-liberated wood pulp in an alkaline aqueous solution under a pressure of 110

oxygenating gas materially greater than the vapor pressure of the solution while said suspension is being agitated.

3. A process which comprises oxygenating a suspension of cellulose fiber in the physical condition of pre-liberated wood pulp in a heated alkaline aqueous solution under a pressure of oxygenating gas materially greater than the vapor pressure of the solution.

4. A process which comprises oxygenating a suspension of cellulose fiber in the physical condition of pre-liberated wood pulp in an alkaline aqueous solution at elevated temperature under a pressure of oxygenating gas materially greater than the vapor pressure of the solution while said suspension is being agitated.

5. A process which comprises confining a suspension of cellulose fiber in the physical condition of pre-liberated wood pulp in an alkaline solution in contact with an atmosphere of oxygenating gas under pressure until the solution viscosity of such fiber has been reduced to below 1.

6. A process which comprises confining a suspension of cellulose fiber in the physical condition of pre-liberated wood pulp in a caustic soda solution in contact with air under a pressure of about 20 to 100 pounds.

7. A process which comprises confining a suspension of cellulose fiber in the physical condition of pre-liberated wood pulp in a dilute, heated, caustic soda solution in contact with an atmosphere of oxygenating gas under pressure.

8. A process which comprises confining a suspension of cellulose fiber in the physical condition of pre-liberated wood pulp in a dilute caustic soda solution at temperatures below about 150° F., in contact with an atmosphere of oxygenating gas under pressure.

9. A process which comprises confining cellulose fiber in the physical condition of pre-liberated wood pulp suspended in an alkaline solution containing metal compounds in contact with an atmosphere of oxygenating gas under pressure.

10. A process which comprises confining cellulose fiber suspended in an alkaline solution containing iron compounds in contact with an atmosphere of oxygenating gas under pressure.

11. A process which comprises confining cellulose fiber in the physical condition of pre-liberated wood pulp suspended in an alkaline solution containing iron compounds in contact with an atmosphere of oxygenating gas under pressure, and removing the iron stain from the resulting product.

12. A process which comprises confining cellulose fiber in the physical condition of pre-liberated wood pulp suspended in an alkaline solution containing iron compounds in contact with an atmosphere of oxygen-

ating gas under pressure, and treating with oxalic acid solution to remove the iron stain from the resulting product.

13. A process which comprises suspending cellulose fiber in the physical condition of pre-liberated wood pulp in an alkaline solution containing bleach, and when the bleach has been substantially consumed subjecting the pulp suspension to the action of oxygenating gas under pressure.

14. A process which comprises treating unbleached pulp with a bleach liquor containing sufficient alkali to maintain a condition of distinct alkalinity throughout the bleaching operation, and after the bleach has been substantially consumed raising the temperature of the pulp suspension and subjecting it to the action of oxygenating gas under pressure.

15. A process which comprises treating cellulose fiber with a caustic soda solution of mercerizing strength, ageing the treated fiber to effect a depolymerization thereof, washing the fiber, and oxygenating the product while suspended in an alkaline aqueous solution under a pressure of oxygenating gas materially greater than the vapor pressure of the solution.

16. A process which comprises treating cellulose fiber with a caustic soda solution of mercerizing strength, ageing the treated fiber to effect a depolymerization thereof, washing the fiber, digesting the fiber in an alkaline solution, and oxygenating the product while suspended in an alkaline aqueous solution under a pressure of oxygenating gas materially greater than the vapor pressure of the solution.

17. A process which comprises treating cellulose fiber with a caustic soda solution of mercerizing strength, ageing the treated fiber to effect a depolymerization thereof, washing the fiber, and oxygenating the product while suspended in a heated, alkaline aqueous solution under a pressure of oxygenating gas materially greater than the vapor pressure of the solution.

18. A process which comprises oxygenating a suspension of cellulose fiber in the physical condition of pre-liberated wood pulp in an alkaline aqueous solution under a pressure of oxygenating gas materially greater than the vapor pressure of the solution while maintaining the suspension in agitation during such oxygenation.

19. A process which comprises oxygenating a suspension of cellulose fiber in a mercerizing solution under a pressure of oxygenating gas greater than the vapor pressure of the solution.

20. A process which comprises suspending an unbleached cellulose pulp in a distinctly alkaline solution containing sufficient bleach to whiten the pulp, and after the bleach has been substantially consumed oxygenating the suspension under a pressure of oxygenat-

ing gas greater than the vapor pressure of the solution.

21. A process which comprises oxygenating a suspension of cellulose fiber in the physical condition of pre-liberated wood pulp in an alkaline aqueous solution under a pressure of oxygenating gas materially greater than the vapor pressure of the solution, and then converting the resulting product of low solution viscosity into cellulose compounds.

10 In testimony whereof I have affixed my signature.

GEORGE A. RICHTER.

15

20

25

30

35

40

45

50

55

60

65